

## [54] METHOD FOR WASHING A TOW

[75] Inventor: Ernest A. Taylor, Jr., Decatur, Ala.

[73] Assignee: Monsanto Company, St. Louis, Mo.

[22] Filed: Dec. 18, 1972

[21] Appl. No.: 315,951

## Related U.S. Application Data

[63] Continuation-in-part of Ser. No. 198,780, Nov. 15, 1971, abandoned, which is a continuation-in-part of Ser. No. 51,261, June 30, 1970, abandoned.

[52] U.S. Cl. .... 8/137.5, 8/137, 134/15

[51] Int. Cl. .... D01f 7/06

[58] Field of Search .... 8/137, 137.5; 134/15

## [56] References Cited

## UNITED STATES PATENTS

|           |         |                      |         |
|-----------|---------|----------------------|---------|
| 2,733,121 | 1/1956  | Griffith, Jr. et al. | 8/137.5 |
| 2,768,057 | 10/1956 | Friederick           | 8/137.5 |

Primary Examiner—Mayer Weinblatt

Attorney, Agent, or Firm—Robert L. Broad, Jr. et al.

[57]

## ABSTRACT

A method for washing a tow wherein the tow is passed through a confined zone and a stream of water is forced through the tow at a minimum rate at least as great as

$$x = 1,000T \sqrt{WN/h} (\mu/\rho)$$

where  $x$  is the water flow rate in gallons per minute,  $T$  is the thickness of the stream of water in inches,  $W$  is the width of the confined zone in inches,  $h$  is the thickness of the confined zone in inches,  $N$  is the number of filaments in the tow,  $\mu$  is the viscosity of the water in pounds per foot-second, and  $\rho$  is the density of the water in pounds per cubic foot. Preferably, the water is forced through the tow at a rate at least 3 times the minimum rate.

13 Claims, 3 Drawing Figures





FIG. 1.



FIG. 2.



FIG. 3.

## METHOD FOR WASHING A TOW

This is a continuation-in-part of application Ser. No. 198,780, filed Nov. 15, 1971, which was a continuation-in-part of application Ser. No. 51,261, filed June 30, 1970 for "Method For Washing A Tow" in the name of Ernest A. Taylor, Jr. both now abandoned.

## BACKGROUND OF THE INVENTION

Man-made fibers are formed by extruding a spinning solution through a spinnerette to form a tow made up of a number of individual filaments. In the production of certain man-made fibers it is usually necessary that this tow be washed during some state of the manufacture. The washing may be for the purpose of removing a spinning solvent, applying a dye or finish, removing excess dye after a dyeing operation, neutralizing the fiber or for some other purpose. Conventionally, the tow is washed by passing it through a spray or a bath or by running it through an inclined cascade in a direction counter to the flow of water in the cascade. These approaches are inefficient, so that the tow must be run through the washing zone at a very low speed or the washing zone must extend a considerable length along the tow processing line. The former lowers the production rate while the latter requires the use of an excessive amount of space which might be better used for some other purpose.

Apparatus other than cascades and sprays has been used to wash tows of filaments. U.S. Pat. No. 3,267,704, issued to H. G. Mueller, and U.S. Pat. No. 3,343,383, issued to E. A. Taylor, Jr., for example, show apparatus used for carrying out the process wherein the washing liquid is continually passed back and forth through the tow until the washing is completed. Unfortunately, the apparatus necessary to carry out this method is usually several feet long and quite expensive to manufacture.

It has been discovered that confining the tow and the washing liquid to a zone having predetermined dimensional limitations and then forcing the liquid through the tow at a rate based on the dimensions of the confined zone and the number of filaments in the tow a vastly superior washing result is obtained. In carrying out the method of the present invention a very simple and inexpensive apparatus may be used, with the complete washing action being carried out in an apparatus no more than five or six inches long. With this in mind, one of the objects of this invention is to provide a novel and improved method for washing a tow of filaments.

Another object of this invention is to provide a method for washing a tow of filaments in such a manner that excess dye or solvent is rapidly and efficiently removed from the tow.

A further object of this invention is to provide a method for washing a tow of continuous filaments in such a manner that the filaments are completely washed within a very short contact time.

A still further object of this invention is to assure a uniform washing of a tow of filaments.

Some tow washing devices operate much more effectively when the washing fluid is boiling, the stirring effect of the ebullient fluid serving to agitate, vibrate or separate the filaments of a tow during washing. Since in this invention a very effective filament separation is produced by the interaction of the fluid with the tow,

then another object of this invention is to eliminate a high fluid temperature as a prerequisite for effective washing.

The objects of this invention are achieved by passing tow to be washed through a confined zone and forcing a stream of water or other treatment fluid through the tow at a rate in excess of a predetermined critical minimum value, the water being maintained at a temperature within a predetermined range. The critical minimum rate at which the water is passed to the tow must be at least as great as

$$x = 1,000T \sqrt{WN/h} (\mu/\rho)$$

where  $x$  is the water flow rate in gallons per minute,  $T$  is the thickness of the stream of water in inches,  $W$  is the width of the confined zone in inches,  $h$  is the thickness of the confined zone in inches,  $N$  is the number of filaments in the tow,  $\mu$  is the viscosity of the water in pounds per foot-second, and  $\rho$  is the density of the water in pounds per cubic foot. Preferably, the water is forced through the tow at a rate at least three times as great as the critical minimum rate.

Other objects and advantages of the invention will become apparent when the following detailed description is read in conjunction with the appended drawing, in which

FIG. 1 is a diagrammatic longitudinal cross-sectional view of one apparatus useful for carrying out the process of the present invention.

FIG. 2 is a cross-sectional view taken along line 2-2 of FIG. 1 showing the cross-sectional area of the confined zone in the washing apparatus through which the tow is passed, and

FIG. 3 is a diagrammatic view of apparatus used with the washing apparatus in carrying out the process of the present invention.

Referring now in detail to the drawing there is shown, in a more or less diagrammatic manner, a tow washer 10 which is useful in carrying out the method of the present invention. The washer 10 is made up of upper and lower units 11 and 12 which are held in a spaced relationship by side plates 13, the side plates 13 being secured to the upper and lower units 11 and 12 by screws 14. The space between the upper and lower units 11 and 12 forms a confined zone through which a tow 15 passes. The lower face 18 of the upper unit 11 and the upper face 19 of the lower unit 12 and the inner faces 20 of the side plates 13 define the limits of the confined zone through which the tow 15 passes. The confined zone thus has a width "W" and a height "h" and a cross section area of  $Wh$ , as best shown in FIG. 2.

The lower unit 12 is provided with an inlet 21 through which water or some other liquid is applied to the tow 15. The inlet 21 extends across the lower unit 12 from one of the side plates 13 to the other and thus has a width  $W$ . The inlet 21 has a thickness of  $AT$ , where  $A$  is between 0.05 and 10, with  $T$  usually being no greater than about  $10h$ ,  $h$  being the height or thickness of the confined zone, so as to concentrate the flow of the washing liquid through the tow 15 at one location. The upper unit 11 is provided with a recess or chamber 22 which receives the water passing through the tow 15 from the inlet 21.

The recess 22 directs the water back through the tow at outlets 23 spaced from the inlet 21 in streams having a thickness  $T$  (FIG. 1), the value of  $T$  preferably being

no greater than about  $10h$ . The preferred value for the dimension  $T$  is within the range of  $2h$  to  $5h$ . The water entering the inlet 21 passes through the tow 15 and is divided into substantially equal parts which pass back through the tow at the outlets 23. The chamber 22 completely fills with water under pressure. This pressure forces the water through the outlets 23, and the tow 15, at a high velocity.

It can readily be seen that the tow is confined, at the outlets 23, to a cross sectional area having the dimensions  $W$  and  $h$ . The fluid passing through the tow at this point is confined to a cross sectional area having the dimensions  $W$  and  $T$ ,  $W$  being width and  $T$  being thickness of the fluid stream.

As shown in FIG. 3, the washer 10 is mounted over a discharge pan 30. Spaced pairs of rolls 32 and 33 feed the tow 15 through the washer 10 at a uniform speed. A pump 34 connected to the pan 30 and the inlet 21 of the washer 10 pumps the water from the pan 30 through the washer via the inlet 21. The water exiting from the washer 10 falls into the pan 30 and is recirculated by the pump through the washer. Fresh water may be fed to the pan 30 from a supply 38, the pan 30 being provided with an overflow line 39 to maintain a constant water level in the pan 30. The fresh water supply rate is independent of the rate at which water is circulated through the washer 10. Pairs of stripper bars 36 positioned in contact with the tow as shown in FIG. 3 are used to prevent the water from flowing along the tow beyond the edges of the pan 30.

The water makes one pass through the tow 15 at each of the outlets 23, for a total of two passes at the outlets. Since twice as much water passes through the tow at the inlet 21 as at either of the outlet locations it may be considered that the water makes a double pass, or two passes, through the tow 15 at the inlet 21. Thus, in the apparatus shown it may be said that the water makes four passes through the tow 15. The water can be deflected back and forth through the tow as many times as desired but the method is so efficient that this is not necessary. At each point where the water passes through the tow the water should be, for maximum efficiency, flowing at a rate in excess of the minimum value given by

$$x = 1,000T \sqrt{WN/h} (\mu/\rho)$$

as set out above. If the water passes through the tow at a lower rate the washing efficiency will be greatly reduced. If a vigorous washing is not required the dimensions of the apparatus 10 may be such that the critical minimum flow rate is exceeded at only one of the outlets 23. In this case the washing will be highly effective only at that outlet.

Of course, a portion of the water in a washer such as described above will not pass completely through the tow but will travel along the interstices in the tow (i.e., between the filaments) to the outlets 23. Since it would be very difficult to actually measure the water flow rate inside the tow an easier way of determining whether the minimum flow rate is exceeded is desired. If the outlet dimensions are held within the limits set out above, the flow rate into the inlet 21 can be compared with the minimum critical flow rate.

$$x = 1,000T \sqrt{WN/h} (\mu/\rho)$$

to determine whether minimum critical flow rate is ex-

ceeded, without regard for actual flow rate in the tow or the fact that some of the water will travel along voids in the tow. Of course, since the one inlet supplies two outlets, the fluid flow into the inlet must be at least twice the critical minimum flow rate as determined by the above equation.

The table below shows values of  $\mu$  and  $\rho$  for water at various temperatures.

| Temperature °C. | lbs/ft-sec.           | lbs/cu. ft. |
|-----------------|-----------------------|-------------|
| 30              | $5.38 \times 10^{-4}$ | 62.16       |
| 35              | $4.85 \times 10^{-4}$ | 62.06       |
| 40              | $4.40 \times 10^{-4}$ | 61.95       |
| 45              | $4.02 \times 10^{-4}$ | 61.82       |
| 50              | $3.69 \times 10^{-4}$ | 61.68       |
| 55              | $3.40 \times 10^{-4}$ | 61.54       |
| 60              | $3.15 \times 10^{-4}$ | 61.38       |
| 65              | $2.92 \times 10^{-4}$ | 61.22       |
| 70              | $2.72 \times 10^{-4}$ | 61.04       |
| 75              | $2.55 \times 10^{-4}$ | 60.86       |
| 80              | $2.39 \times 10^{-4}$ | 60.67       |
| 85              | $2.25 \times 10^{-4}$ | 60.47       |
| 90              | $2.12 \times 10^{-4}$ | 60.27       |
| 95              | $2.01 \times 10^{-4}$ | 60.05       |
| 100             | $1.90 \times 10^{-4}$ | 59.83       |

The following examples are included to show the efficiency of this tow washing process in removing solvent from wet spun acrylonitrile filaments. Four washers (not shown) such as described above were used in series, with the freshly spun tow entering washer A and then passing through washers, B, C and D in that order. Each washer formed a confined zone 5.2 inches long and having the dimensions:  $T = 9/16''$ ;  $h = 3/16''$  and  $W = 3 - 7/8''$ . Each washer was provided with its own pan or reservoir 30 from which wash water at  $50^\circ\text{C}$ . was circulated through the washer at a rate in excess of the critical minimum flow rate as determined by the equation given above.

Fresh water was supplied to washer D from its supply 38 and the overflow line 39 of washer D was connected to feed this overflow into the pan 30 of washer C. The overflow of washer C fed into washer B from which the overflow fed into the pan 30 of washer A. The overflow of washer A was passed to a solvent recovery system (not shown). The fresh water supply rate, which is independent of the circulation rate in each of the washers, was based on the weight of the tow passing through the washers and was varied as shown in the following examples.

The tow was spun from a 93% acrylonitrile, 7% vinyl acetate copolymer into a spin bath of 55% dimethylacetamide/45% water at  $38^\circ\text{C}$ . and was led from the spin bath into washer A. The tow entering washer A contained about 50% dimethylacetamide. The tow was made up of 80,000 filaments, 3 denier per filament. The tow was advanced at a speed such that a given point on the tow passed through the confined zone in 0.95 seconds. This may be referred to as "contact time" or "dwell time."

#### EXAMPLE I

Tow was spun at a rate of 600 pounds per hour. The values given under the headings A, B, C and D represent the amount of solvent in the tow exiting from the washers A, B, C and D, respectively.

| Fresh Water Supply Rate lb H <sub>2</sub> O/lb tow | Solvent in tow % by weight |      |      |      |
|----------------------------------------------------|----------------------------|------|------|------|
|                                                    | A                          | B    | C    | D    |
| 12.5                                               | 7.44                       | 1.30 | 0.45 | 0.25 |
| 10.3                                               | 7.75                       | 2.35 | 0.64 | 0.22 |

## EXAMPLE II

Tow was spun at a rate of 735 pounds per hour. Fresh water was added to the reservoir or pan 30 of washer D at varying rates and the amount of solvent in the tow after each washer was determined. The results are shown in the following table.

| Fresh water Supply Rate lb H <sub>2</sub> O/lb tow | Solvent in tow % by weight |      |      |      |
|----------------------------------------------------|----------------------------|------|------|------|
|                                                    | A                          | B    | C    | D    |
| 12.5                                               | 8.86                       | 2.67 | 0.85 | 0.34 |
| 8.3                                                | 11.63                      | 3.38 | 0.84 | 0.39 |

The temperature of the water used for washing may

| Fiber                                          | Polyvinyl Chloride |      |      |      |     | Polyester |     |     | Nylon |     |     | Rayon |     | Polyester |       |
|------------------------------------------------|--------------------|------|------|------|-----|-----------|-----|-----|-------|-----|-----|-------|-----|-----------|-------|
|                                                | 1                  | 2    | 3    | 4    | 5   | 6         | 7   | 8   | 9     | 10  | 11  | 12    | 13  | 14        | 15    |
| Run No.                                        |                    |      |      |      |     |           |     |     |       |     |     |       |     |           |       |
| Tow speed entering confined zone (ft/min)..... | 39.5               | 20.0 | 59.0 | 10   | 40  | 50        | 60  | 10  | 40    | 10  | 40  | 20    | 40  | 10        | 40    |
| Tow speed leaving confined zone (ft/min).....  | 156                | 78.0 | 235  | 56.8 | 180 | 205       | 240 | 52  | 162.5 | 45  | 180 | 25    | 45  | 52        | 202.5 |
| Time in confined zone (seconds).....           | 0.6                | 1.3  | 0.4  | 2.4  | 0.6 | 0.5       | 0.4 | 2.4 | 0.6   | 2.4 | 0.6 | 1.8   | 0.9 | 2.4       | 0.6   |
| Stretch Ratio.....                             | 4                  | 4    | 4    | 5.6  | 4.5 | 4.0       | 4.0 | 5.2 | 4     | 4.5 | 3.5 | 1.25  | 1.1 | 5.2       | 5     |

be up to 100° C. The preferred temperature for washing acrylonitrile filaments to remove solvent is within the range of 30° C. to 70° C.

## EXAMPLE III

A freshly spun modacrylic tow was washed in a confined zone having the following dimensions:  $W - 3\frac{1}{2}$  inches;  $h - 7/32$  inches; and  $T - 9/16$  inches. The tow bundle contained 6,000 filaments of 50 denier each. The fibers in the tow had the following composition: Acrylonitrile 60.6%, Vinylidene Chloride 23.0%, Vinyl Bromide 11.0%, Styrene 1.4%, Benzene Sulfonate 2.0% and Antimony Trioxide 2.0%.

Water at a temperature of 96° C. and containing 4% sodium phosphate was used for washing the fiber. The liquid flow rate was in excess of three times the critical minimum value and the time of the tow in the treatment zone was approximately 1.5 seconds. The filaments in the tow were neutralized from a pH of 3.9 to a pH of 8.5.

## EXAMPLE IV

The modacrylic tow of Example III was washed in water at 50° C. in a confined zone having the dimensions of Example III. A conventional dye, known to be suitable for the dyeing of modacrylic fibers, was substi-

tuted for the sodium phosphate in an amount sufficient to provide a dye concentration of 0.5% based on the weight of the water. The liquid flow rate was in excess of three times the critical minimum value and the time of the tow in the treatment zone was approximately 1.5 seconds. The filaments in the tow were dyed to a deep, uniform shade. The amount of dye on the fiber was approximately 2%, based on the weight of the fiber.

## EXAMPLE V

A number of runs were made using filaments of different chemical composition wherein the filaments were washed with water containing a finish for the purpose of applying the finish to the filaments. Fiber types included in these runs were polyvinyl chloride, polyester, nylon and rayon, all well known to those skilled in the art. The washing fluid was 98% water and 2% of a conventional finish, at a temperature of 100° C. In addition to being washed, the filaments were stretched.

The confined zone had the following dimensions:  $W - 3/16$ ";  $h - 3/16$ "; and  $T - 9/16$ ", with an overall length of 8". The number of filaments in each bundle of filaments passing through the confined zone was such that the minimum critical flow rate varied up to approximately 0.1 gallon per minute for the different fibers. The actual flow rate through the confined zone was 1.2 gallons per minute. The following table shows the conditions under which these runs were made. Approximately 1% of the finish, based on the weight of the fiber, was applied to the fiber in each washing run.

| Fiber                                          | Polyvinyl Chloride |      |      |      |     | Polyester |     |     | Nylon |     |     | Rayon |     | Polyester |       |
|------------------------------------------------|--------------------|------|------|------|-----|-----------|-----|-----|-------|-----|-----|-------|-----|-----------|-------|
|                                                | 1                  | 2    | 3    | 4    | 5   | 6         | 7   | 8   | 9     | 10  | 11  | 12    | 13  | 14        | 15    |
| Run No.                                        |                    |      |      |      |     |           |     |     |       |     |     |       |     |           |       |
| Tow speed entering confined zone (ft/min)..... | 39.5               | 20.0 | 59.0 | 10   | 40  | 50        | 60  | 10  | 40    | 10  | 40  | 20    | 40  | 10        | 40    |
| Tow speed leaving confined zone (ft/min).....  | 156                | 78.0 | 235  | 56.8 | 180 | 205       | 240 | 52  | 162.5 | 45  | 180 | 25    | 45  | 52        | 202.5 |
| Time in confined zone (seconds).....           | 0.6                | 1.3  | 0.4  | 2.4  | 0.6 | 0.5       | 0.4 | 2.4 | 0.6   | 2.4 | 0.6 | 1.8   | 0.9 | 2.4       | 0.6   |
| Stretch Ratio.....                             | 4                  | 4    | 4    | 5.6  | 4.5 | 4.0       | 4.0 | 5.2 | 4     | 4.5 | 3.5 | 1.25  | 1.1 | 5.2       | 5     |

This process may be used not only to remove solvent from a freshly spun tow but also may be used for other washing such as application of a dye or finish or removal of excess dye after a dyeing process, etc. The washing efficiency becomes unsatisfactory if the flow rate through the washing zone is not maintained above the critical minimum value as set out above. Preferably, the flow rate is at least three times the minimum rate and may be many times as great as the minimum rate.

The minimum dwell or contact time of the tow in the confined zone (i.e., the length of time that a given point on the tow requires to pass through the fluid in the confined zone) varies slightly with the washing operation. For example, if it is desired to wash the tow to apply a finish, a contact time of about 0.1 second or more is all that is required. If the washing is done to remove solvent from a freshly spun tow a contact time of 0.25 seconds or more should be used.

What is claimed is:

1. The method of washing a tow of filaments, comprising
  - a. advancing the tow through a confined zone, and
  - b. forcing a stream of liquid through the tow in the confined zone at a rate greater than

$$x = 1,000 T \sqrt{WN/h} (\mu/\rho)$$

where  $x$  is the liquid flow rate in gallons per minute,  $T$  is the thickness of the stream of liquid in inches,  $W$  is the width of the confined zone in inches,  $h$  is the height of the confined zone in inches,  $N$  is the number of filaments in the tow,  $\mu$  is the viscosity of the liquid in pounds per foot-second, and  $\rho$  is the density of the liquid in pounds per cubic foot.

2. The method of claim 1 wherein the liquid is forced through the tow in the confined zone at a rate at least three times as great as

$$x = 1,000T \sqrt{WN/h} (\mu/\rho)$$

3. The method of claim 2 wherein the liquid makes at least four passes through the tow.

4. The method of claim 2 wherein the temperature of the liquid is in the range of 30° C. to 100° C.

5. The method of claim 2 wherein the filaments are acrylonitrile.

6. The method of claim 2 wherein the filaments are modacrylic.

7. The method of claim 2 wherein the filaments are polyester.

8. The method of claim 2 wherein the filaments are nylon.

9. The method of claim 2 wherein the filaments are rayon.

10. The method of claim 2 wherein the tow is ad-

vanced through the confined zone at a speed such that the tow is in contact with the liquid stream for at least 0.1 seconds.

11. The method of washing a tow of filaments, comprising,

a. passing the tow through a washing zone, said zone confining the tow in such a manner that the tow has a cross-sectional area having a width  $W$  and a height  $h$ ,

10 b. forcing a stream of liquid through the tow in said washing zone, said stream of liquid having a width  $W$  and a thickness  $T$  and also having a flow rate greater than

$$1,000T \sqrt{WN/h} (\mu/\rho)$$

where  $N$  is the number of filaments in the tow,  $\mu$  is the viscosity of the liquid in pounds per foot-second, and  $\rho$  is the density of the liquid in pounds per cubic foot.

20 12. The method of claim 11 wherein the flow rate is at least three times

$$1,000T \sqrt{WN/h} (\mu/\rho)$$

13. The method of claim 12 wherein the filaments are selected from the group consisting of acrylic, modacrylic, nylon, polyester, polyvinyl chloride and rayon.

\* \* \* \* \*